

1,036,500.

F. B. LAMB.  
METALLURGICAL FURNACE.  
APPLICATION FILED SEPT. 21, 1911.

Patented Aug. 20, 1912.

4 SHEETS—SHEET 1.

FIG. 1.



Witnesses

John H. Smith  
E. Lundy

Inventor  
Fred B. Lamb

By Frank D. Thoreson  
Attest

1,036,500.

F. B. LAMB.  
METALLURGICAL FURNACE.  
APPLICATION FILED SEPT. 21, 1911.

Patented Aug. 20, 1912.  
4 SHEETS-SHEET 2.

FIG. 2.



Witnesses  
Ollie Nequin  
E. Lundby.

Inventor  
Fred B. Lamb  
by Frank D. Thompson  
Atty

1,036,500.

F. B. LAMB.  
METALLURGICAL FURNACE.  
APPLICATION FILED SEPT. 21, 1911.

Patented Aug. 20, 1912.

4 SHEETS—SHEET 3.



Witnesses  
O. M. Knudsen  
S. Kennedy

Inventor  
Fred B. Lamb  
by Frank D. Hanaway  
Atty.

1,036,500.

F. B. LAMB.

METALLURGICAL FURNACE.

APPLICATION FILED SEPT. 21, 1911.

Patented Aug. 20, 1912.

4 SHEETS—SHEET 4.



FIG. 2.

Witnesses.  
O. M. Kunkel  
E. P. Lundy.

Inventor  
Fred B. Lamb  
by Frank D. Thompson  
atty.

# UNITED STATES PATENT OFFICE.

FRED B. LAMB, OF BETTENDORF, IOWA, ASSIGNOR OF ONE-FOURTH TO ALBERT B. FRENIER, OF DAVENPORT, IOWA.

## METALLURGICAL FURNACE.

1,036,500.

Specification of Letters Patent. Patented Aug. 20, 1912.

Original application filed February 28, 1911, Serial No. 611,409. Divided and this application filed September 21, 1911. Serial No. 650,494.

To all whom it may concern:

Be it known that I, FRED B. LAMB, a citizen of the United States, residing at Bettendorf, in the county of Scott and State of Iowa, have invented new and useful Improvements in Metallurgical Furnaces, of which the following is a full, clear, and exact description.

This application is a division of my original application No. 611,409 filed February 28th, 1911.

The invention embodies a modified form of the class of furnaces generally known as the tilting open hearth furnace of the regenerative type, to which has been added a "receiving" or converting chamber.

The principal object of my invention is to combine in a single unit the well known open hearth furnace with an ordinary condenser, in a manner that when used for making steel, the recognized and time-proven superior features only, of each device is to be utilized—limiting the use of each to that which it accomplishes best, quickest, cheapest and with the least damage to itself and minimum waste of materials.

Another object of my invention is to greatly increase the capacity of a steel furnace and permit the use of raw materials of a chemical content heretofore considered prohibitive, yet bringing forth a high grade of steel with a degree of economy heretofore impossible. This I accomplish in the manner hereinafter fully described and as particularly pointed out in the claims.

In the drawings: Figure 1 is a transverse section of a tilting furnace embodying my improvements. Fig. 2 is a similar view showing the furnace tilted toward the converter. Fig. 3 is a similar view showing the furnace tilted in the opposite direction for "pouring." Fig. 4 is a view showing one-half of the furnace in longitudinal central section and the other half in side elevation.

The open hearth furnace is unquestionably the fastest and most economical means known for liquefying a cold charge, and when basic lined it is unexcelled for the elimination of phosphorus. The converter either of the "bottom," "side" or "surface" blow type excels in the rapid elimination of carbon and silicon. I have therefore designed a furnace in which will be found combined, in a single unit, the tilting open

hearth and the converter so arranged and coöperating in such a manner that the superior features only of each individual furnace is to be utilized—using only those features that contribute to the saving of time, labor and fuel, eliminating the more expensive and long drawn out operations which cannot be separated from those devices when used separately. This kind of a furnace comprises a substantially rectangular body having a front wall A, a rear wall B, end walls C, a bottom D and a roof R. The bottom or floor consists of a supporting metal retaining sheet a, which, between its parallel upwardly flanged side edges is concaved or dished and provided with the ordinary silica brick b, which, in turn, is covered with the material c, for either an acid or basic lined bottom. The sheet a is reinforced both longitudinally and transversely, and near its ends it is provided with corresponding rockers d. The curved treads of these rockers rest and travel upon a series of segmentally arranged anti-friction rollers, e, that are journaled at equal distances apart in parallel segmental frames e', and these rollers rest and travel upon concaved tracks E built upon a suitable foundation. The end walls C of the furnace are provided with the usual gas or fuel ports F, through which the gas from the burner H and heat from the regenerative chambers (not shown) through the flues h are blown into the furnace. The curved treads of the rockers d, and the concaved tracks E are struck from an axis intersecting the center of the fuel ports, so that, no matter in what tilted position the furnace may be, the heat products will continue to blow into the furnace.

The furnace may be tilted or rolled through the medium of a hydraulic cylinder G having a ram or piston f, which connects with the center of length of one of the rockers, at a point above its tread.

The front wall A of the furnace is provided with the usual charging doors. The lower portion, of the central charging door is formed by the bottom of the furnace being extended out under this doorway forming the bottom of a pouring spout J, the side edges of which are raised sufficiently to confine the metal when pouring. This charging doorway is opened and closed by a vertically movable gate K, which is

operated through the medium of a chain or cable by suitable mechanism (not shown).  
 Opposite the charging door-way, the rear wall of the furnace is provided with a comparatively small opening 2, which communicates with a blowing chamber or converter 3 at a point next the bottom thereof, which latter and the floor of said opening are a continuation of the bottom of the furnace.  
 This "blowing chamber" or converter 3 is built out from and removably attached to the rear wall of the furnace. Its outer shell may be of rectangular shape and is made of sheet metal. It is lined by a course of brick and by an inner lining of the composition usually employed for lining converters. The inner contour of the inner lining is of flask shape with the mouth or opening drawn to one side as shown. This converter is retained in place against the rear wall of the furnace by any suitable means, such as lugs and key-wedges (not shown). Its outer wall terminates below the plane of the inner wall, and is constructed so that slag from the metal therein can be drawn or blown off, as will hereinafter more fully appear. The upper part of the inner wall is built out so as to overhang, forming a partial roof of the converter. At the bottom the inner wall is provided with an opening, which is made to register with opening 2 in the rear furnace wall when converter is clamped thereto. The bottom of the converter is provided with a series of openings or tuyers 5, communicating with an air-chest or box 6, that is supplied with air under pressure from an air intake 7. A vertical passage 8 is provided in the rear wall of furnace immediately above and separate from opening 2. Its lower end is projected outward and discharges into the converter through a suitably provided opening. If desired a suitable air blast pipe may extend down through this passage, through which a blast of air may be blown, or the passage may be suitably prepared for doing this. While a "bottom blow" converter is thus shown and described, it is evident that a "side blow" or a "surface blow" type of converter could be used.

While the open hearth furnace of the present day practice, when lined basic, removes or reduces to within allowable limits, carbon, silicon, manganese, phosphorus and possibly sulfur, the length of time, and amount of labor, fuel and expense required to make the proper reduction, depends altogether upon the manner in which the above elements are chemically combined. If the cold charge be high in carbon, liquefaction begins promptly and the entire mass is melted down quickly, but the attending reduction of the carbon to within the allowable limits is accomplished only after several hours of painstaking labor and the subjec-

tion of the bath to the fierce oxidizing action of the fuel. If sulfur is also present further time must be expended and more fuel consumed in what oft times proves a futile attempt to remove it. While it is possible to bring forth a very satisfactory grade of steel from the basic open hearth furnace, the baser the raw materials, the more difficult and more expensive does the operation become and the more damaging to the furnace, due to the long exposure to the fierce action of the fuel, necessitating more frequent and expensive repairs and greatly increased cost of maintenance. Confining its use to that which it accomplishes quickest and best, namely, melting and dephosphorizing, leaving the reduction of carbon and silicon to other means, the first step toward lowering cost of production is achieved. As the open hearth excels in melting and dephosphorizing so does the converter excel in removing carbon and silicon. My improved furnace combines these two well known agencies and their individually superior functions are so manipulated that the highest grade of steel is brought forth from materials and at a cost heretofore impossible.

The operation of my improved furnace is substantially as follows: After the hearth or melting chamber, which is lined basic, has been raised to the proper temperature, limestone is charged to form a slag, then 15 tons (presuming the furnace to be of 15 tons capacity) of cheap low grade pig iron, or part pig and part steel scrap, or all cast scrap or cast borings. As the carbon content of an all pig charge or of a cast scrap would be very high, liquefaction will begin promptly and the entire charge will be melted down in about two hours. While a regular open hearth furnace would melt this high carbon charge just as quickly, the attending reduction of this carbon and silicon to within allowable limits can only be accomplished at the expense of much labor and hours of time. It is this feature of steel making by the open hearth that creates expense and contributes to the high cost of the finished product. If metal of lower carbon be charged into an open hearth furnace, such as half pig and half scrap, it will naturally take less time and expense to reduce the carbon to within allowable limits, but this gain will be offset by the increased time taken to melt, so that what is saved in one direction is lost in another. In order to keep carbon and sulfur low as possible, half select pig and half select steel scrap are usually used in open hearth practice. This is high priced material. A low grade cheap pig iron could be used at a great saving, if its first cost were not offset by the excessive expense incurred in reducing carbon and other injurious elements. In my improved furnace the open hearth department will not be called

upon to perform this expensive part of the process, but confined solely to melting and dephosphorizing, for, as soon as about 5-tons of melted metal has accumulated in the bath, the blast will be turned into the converting chamber 3 (if it be a "bottom blow" converter as shown) and the furnace tilted toward the converter until it is nearly, but not quite, in the position shown in Fig. 2 of the drawings, and the molten metal will flow through the opening 2 into same. In about ten minutes this five-ton mass of molten metal will be thoroughly decarbonized and desiliconized and incidentally its temperature raised from about 1800° to about 3000°. Thus the converting department of my improved furnace accomplishes in a few minutes that which takes hours by the open hearth furnace, and with no other fuel than a blast of air. In addition to this great saving of time and expense, other most favorable conditions obtain—conditions non-existent in the straight open hearth practice. These are first, a highly acid slag develops during the act of blowing in the converter. This is removed by tilting the furnace farther in the same direction until the level of the surface of the metal reaches the lip or upper edge of the outer wall of the converter, as shown in Fig. 2, so as to allow the slag to drain off. The removal of the slag in this manner may be expedited by directing a blast of air from the mouth of the air passage 8 laterally across the surface of the metal. Thus the bath is freed from a large mass of highly acidulous and impure matter without interrupting the continued action of the furnace, an accomplishment impossible in the regular open hearth furnace. Second. As the furnace is tilted back to its normal position, this 5-tons of metal at a temperature of about 3000° flows back into the melting chamber, intermingling with the bath and materially raising the temperature of the entire mass and greatly hastening the liquefaction of the unmelted portion of the charge at a great saving of fuel. Third. This metal from the converter being thoroughly impregnated with oxidizing gases, due to the action of the air blown into it, the carbon in the bath will most eagerly combine therewith, acting exactly as iron ore does in the ordinary practice, thus effecting another saving in avoiding the use of iron ore as an oxidizing agent. As the furnace has been made to tilt with the gas or fuel ports as an axis, the melting operation in the melting chamber has not been interrupted during the act of "blowing" and returning the "blown" mass to the parent bath. Dephosphorization, through the action of the lime slag has also gone on uninterruptedly. If a test is now made, and it shows "high" carbon, another five tons may be "blown" in a few minutes as before, each time gaining in the

removal of a large portion of highly acidulous slag and in a greatly increased temperature of the bath. At the end of about two hours time the entire charge will be melted, decarbonized, desiliconized, dephosphorized and brought to a very high temperature. The furnace is then tilted in the direction shown in Fig. 3 of the drawings, and the contents drawn off through the pouring spout J into a ladle ready for teeming. 75

I do not confine myself to the production of steel from a cold charge, as "hot" or melted metal from the blast furnace, cupola or mixer can be introduced into the melting chamber of my furnace and the most satisfactory and economical results follow. 80

What I claim as new is:

1. A metallurgical furnace of the open hearth type comprising a melting chamber and a "blowing" chamber outside of and communicating in its lower part with the melting chamber and provided with an outlet disconnected therefrom, and means for tilting the furnace. 85

2. A metallurgical furnace of the open hearth type, comprising a melting chamber, a "blowing" chamber outside of the melting chamber and provided with an outlet separate therefrom, fuel ports and regenerating chamber flues, communicating with the melting chamber and means for tilting the furnace adapted to maintain operative communication between the melting chamber, the "blowing" chamber, fuel ports and the regenerating chamber flues while the furnace is in its normal position, in a tilted position or during the period of tilting. 95

3. A metallurgical furnace having an open hearth provided with fuel ports and communication with regenerative chambers, and a "blowing" chamber outside of and communicating in its lower part with the hearth and having an outlet separated therefrom, and means for tilting the furnace adapted to maintain operative communication between the hearth, the "blowing" chamber, fuel ports and regenerative chamber flues whether the furnace is in a normal position, a tilted position or during the period of being tilted. 110

4. A metallurgical furnace comprising a hearth and a removably attached blowing chamber communicating therewith, and means for tilting the furnace. 115

5. A metallurgical furnace comprising a hearth, a removable blowing chamber exteriorly attached to one of the side walls and communication from the hearth to the blowing chamber, charging doors and pouring spout located in the opposite side wall, end walls and fuel and gas ports communicating with the hearth, and means for tilting the furnace. 120

6. A metallurgical furnace having a hearth, a blowing chamber having commu- 125

130

- nication with the hearth and having an outlet separated therefrom, provided with air blast slag removing means, and means for tilting the furnace.
5. 7. A metallurgical furnace comprising a hearth, a blowing chamber outside of and communicating therewith, and having an outlet separated therefrom, fuel ports at the ends of the hearth communicating with re-
- 10 generative chambers, and means for rocking the furnace about the fuel ports as an axis.
8. A metallurgical furnace comprising an open hearth, a removably attached blowing chamber communicating therewith, fuel ports at the ends of the hearth communicating with regenerative chambers, and means for rocking the furnace about the fuel ports as an axis.
9. A metallurgical furnace of the open
- 20 hearth type, comprising a melting chamber, a blowing chamber exteriorly attached to one of the side walls and having communication with the hearth and provided with an outlet independent thereof, air blast slag removing means in said wall, end walls provided with fuel ports communicating with the hearth and regenerative chambers, and means for tilting the furnace about the fuel ports as an axis.
- 15 10. A metallurgical furnace of the open 30 hearth type, comprising a melting chamber provided with fuel ports and regenerating chambers, a blowing chamber exteriorly attached to and communicating with the melting chamber and means whereby the act of 35 melting in the melting chamber and conversion in the blowing chamber can be performed simultaneously.
11. A metallurgical furnace comprising a hearth provided with fuel ports and regen- 40 erator chambers, a removably attached converter communicating with the hearth, and means whereby the blowing chamber may be operated without interrupting continuous liquefaction in the hearth. 45
12. A metallurgical furnace comprising a hearth provided with fuel ports and regenerative chambers, a removably attached blowing chamber communicating with the hearth, and means whereby the blowing chamber may be removed without interrupting continuous liquefaction in the hearth. 50

In witness whereof I have hereunto set my hand this 18th day of September 1911.

FRED B. LAMB.

Witnesses:

A. B. FRENIER,  
HENRY BELLINGHAUSEN.